

## ABRASIVE ARTICLES AND METHOD OF MAKING

James E. Price, Abington, and Kenneth Deane Groves, Bryn Mawr, Pa., assignors to American Viscose Corporation, Wilmington, Del., a corporation of Delaware

No Drawing. Application October 23, 1951,  
Serial No. 252,792

6 Claims. (Cl. 51—298)

This invention relates to fibrous structures comprising 15 non-fibrous particulate filling materials and fibers at least 50% by weight of which are potentially adhesive cotton fibers having a cellulose ester firmly adhered to their surfaces, fibers in the product being bonded together by the cellulose ester.

In the production of fibers or other shaped articles from cellulose acetate and other fiber-forming organic acid esters of cellulose it is the common practice to filter the ester dope through cotton batting before it is delivered to the spinnerets or other forming devices. As a result of filtering the ester dope, the cotton fibers of the 25 batting are impregnated by the ester, some of which adheres to the fibers. The cotton batting eventually becomes clogged by the retained ester and has to be discarded. Such discarded ester-impregnated filter media have heretofore been regarded as waste.

We have found that although cotton fibers are not per se potentially adhesive fibers and cannot be activated to a tacky or adhesive condition, the non-fibrous cellulose acetate or similar cellulose ester adhering to the surfaces 35 of the fibers of the cotton batting filter is activatable to tacky condition by heat or solvent action after drying of the ester-impregnated batting so that the fibers obtained by grinding the dried batting can be used as a binder for particles of various non-fibrous fillers, for example particles of abrasive materials, to produce molded fibrous products having desirable physical properties.

The products of this invention consist of a matrix constituted by a compacted, felt-like fibrous structure formed of or comprising the cotton fibers having the cellulose acetate adhered to their surfaces and particles of a non-fibrous filling material which are distributed substantially uniformly through the matrix.

The products are made by commingling fibers at least 50% by weight of which are the cotton fibers carrying the cellulose ester and particulate non-fibrous filling materials to obtain an intimate mixture of the fibers and particles in which the latter are in contact with the cellulose ester adhering to the surfaces of the cotton fibers, activating the ester to softened or tacky condition to bind fibers in the product, and deactivating the ester to set the fibers firmly in the bonded relation, the filler particles being held securely in the product by the bonded fibers.

The final product may consist wholly of the cotton fibers carrying the cellulose ester and the filler particles, or it may also contain a small proportion of fibers which are not themselves activatable to the tacky condition and which are not coated or impregnated with an activatable material, as well as other types of fibers which are activatable to tacky condition, i. e., fibers which are potentially adhesive but different from the cotton fibers carrying the ester.

For example, in addition to the filler particles and the cotton fibers coated or impregnated with cellulose acetate or the like, the products may contain a given proportion, that is, up to 50% based on the total weight of the fibers in the product, of natural fibers, such as, for example,

wood fibers, cotton, flax, jute, kapok, wool, hair and silk in their natural non-activatable condition, or it may contain artificial or synthetic fibers including cellulosic fibers such as, for example, cellulose hydrate, cellulose esters and mixed cellulose esters which are non-thermoplastic and not rendered tacky under the conditions used to bind the filler particles and ester-coated cotton fibers together, cellulose ethers, mixed cellulose ester ethers, mixed cellulose ethers, cellulose hydroxy-alkyl ethers, cellulose carboxyalkyl ethers, cellulose ether-xanthates, cellulose xantho-fatty acids, cellulose thiourethanes; natural and synthetic rubber and derivatives thereof; fibers made of alginic acid, gelatine, casein; and mineral fibers such as those of spun glass, asbestos, mineral wool, and the like; and fibers made of natural and synthetic resins which are not rendered tacky under the operating conditions employed, as well as fibers and filaments obtained by slitting, cutting, or shredding non-fibrous films such as cellophane.

20 The potentially adhesive fibers which may be present with the cellulose ester-treated cotton fibers in an amount up to 50% based on the total weight of the fibers in the product, may be composed of a wide variety of materials and may comprise any material capable of being formed into fibers which have an inherent tackiness under conditions such that those fibers and the cellulose ester adhered to the surfaces of the cotton fibers are rendered tacky without damage to the cotton fibers or to any other non-adhesive fibers present, and which are not tacky at room temperature. Examples of the potentially adhesive fibers which may be present are thermoplastic fibers such as those of cellulose acetate or other cellulose esters and ethers, or mixed cellulose esters such as cellulose acetate-propionate or cellulose acetate-butyrate, in plasticized condition; also resins as, for example, cheap natural resins such as shellac, dammar, copal and the like, and synthetic resins which are either permanently thermoplastic or thermosetting but in the thermoplastic state at the time they are mixed with the cellulose-ester coated fibers which 30 are the principal binding fibers in the product, the synthetic resins being formed by the polymerization or condensation of various organic compounds such as coumarone, indene or related hydrocarbons, vinyl compounds, styrene, sterols, aldehydes, fufural, ketones, urea, thiourea; phenol-aldehyde resins either unmodified or modified with oils; urea-aldehyde resins; sulfonamide-aldehyde resins; polyhydric alcohol-polybasic acid resins; drying oil-modified alkyd resins; resins formed by the polymerization of acrylic acid or its homologues or derivatives; sulfur-olefine resins; resins formed from dicarboxylic acids and diamines (nylon type) or from dicarboxylic acids and polyethylene glycols ("Dacron" type); synthetic rubbers and rubber substitutes, herein called "resins," such as, for example, polymerized butadiene, olefine poly-sulfides, isobutylene polymers, chloroprene polymers; polyethylene; and fibers formed from a resin comprising polymeric substances obtained by copolymerizing or interpolymerizing two or more copolymerizable monomers, such as copolymers of a vinyl halide and a vinyl organic acid ester, e. g., copolymers of vinyl chloride and vinyl acetate, copolymers of a vinyl compound and a styrol compound, copolymers of acrylonitrile with one or more other mono-ethylenically unsaturated monomers which are copolymerizable with acrylonitrile, and also a mixture of resins, such as a mixture of poly-olefine resins and phenol-aldehyde resins, or a mixture of two or more resins from the different classes named above. There may be used, also, fibers made from rubber latex, crepe rubber, gutta percha, balata, and the like.

When the products contain fibers other than the cotton fibers having the cellulose ester adhered to their surfaces, the total of such other fibers including both non-adhesive

and potentially adhesive fibers, is not in excess of 50% by weight, based on the total weight of the fibers in the product.

The fibers and particles may be bonded together solely by activation of the cellulose ester on the surfaces of the cotton fibers and of any fibers present in the product which are per se potentially activatable to the tacky or adhesive condition, or the product may also comprise a non-fibrous thermosetting resin which is applied to the mixed fibers and filler particles in liquid condition, and brought to the hardened, thermoset condition in situ in the product. Any of the thermosetting resins commonly used in the molding art may be used but preferably the thermosetting resin is a melamine-formaldehyde resin or a phenol-formaldehyde resin. The choice of the thermosetting resin will depend on the type of fibers mixed with the cellulose ester-treated cotton fibers, if such other fibers are used, since some of the thermosetting resins are more satisfactory for use with certain types of potentially adhesive fibers than with others. For example, when fibers of a potentially adhesive vinyl resin, such as fibers of vinyl chloride-vinyl acetate copolymers are present in addition to the cotton fibers carrying the cellulose ester, it is preferred to avoid the use of phenolic resins as extraneous binders, melamine-formaldehyde resins having been found to be more satisfactory. The use of the melamine-formaldehyde or phenol-formaldehyde resin in conjunction with the cotton fibers having the cellulose ester coating or carrying adhered particles of the cellulose ester on their surfaces improves the strength of the product by reinforcing the bonds between the fibers and between the fibers and filler particles.

The choice of non-fibrous filler for admixture with the fibers will be determined entirely by the purpose for which the final product is intended since the filler will, of course, have a definite effect on the physical properties of the final product. Thus, the filler may serve simply to fill the interstitial spaces between fibers in the product, thereby increasing the density of the product and also increasing its mechanical and impact strength; or it may also improve or modify the properties of the product in other respects, for instance the conductivity of the product for heat or electricity; its resistance to shock or chemical reagents; its abrasiveness, etc. The filler may be a pigment, such as chromium oxide, titanium oxide, iron oxide pigments, barium sulfate, carbon black, graphite, zinc oxide, etc. Further the filler may be a special absorbent substance such as activated magnesium silicate, activated carbon, silica gel, activated alumina, fuller's earth, activated bleaching clay, activated bauxite, French chalk or the like. Or the filler may be a substance such as asbestos powder, mica, sand, rotten stone, clay, brick dust, diatomaceous earth, talcum, slate powder, etc.

In the preferred embodiment of the invention, however, the filler is an abrasive material and the final product is adapted to use as an abrading or polishing device. Any of the abrasives in common use may be used, including silicon carbide, boron carbide, fused aluminum oxide, flint, pumice, Carborundum, emery, rouge, and similar materials. The size of the abrasive particles may vary from the finest polishing or buffing powder to the coarser grit sizes used in grinding.

The cotton fibers having the cellulose ester adhered to their surfaces may be obtained by drying the cotton batting used in filtering the cellulose ester after it has become clogged and useless as a filter, and then grinding, shredding or cutting the batting to produce a mass of loose cotton fibers the surfaces of which are coated with the ester or which have particles or discrete deposits of the cellulose ester firmly adhered to their surfaces.

The filler particles and fibers may be commingled and formed into shaped articles in any suitable manner. For example, the fibers and filler particles may be commingled by blowing them with air or any other gaseous or vaporous but preferably gaseous medium into a common mixing

and depositing chamber, and permitting the thus freely intermixed fibers and particles of filler to settle out on a collecting device.

After association of the fibers and non-fibrous filler particles and collection of the mixture, the product is compacted and the cellulose ester adhering to the surfaces of the cotton fibers, as well as any fibers of the potentially adhesive type present in the mixture, are activated by heat or solvent to effect a firm binding of the fibers and filler particles. After the activation and compaction, which operations may be performed simultaneously, the activated ester film or deposits on the surfaces of the cotton fibers, and any activated fibers present, are deactivated to non-adhesive condition to fix the fibers and filler particles in the new relationship. If activation has been accomplished by heat, deactivation may be effected by heating for a prolonged period or by cooling. If activation is by means of a solvent for the cellulose ester, for instance acetone in the case of cellulose acetate, deactivation may involve extraction of the solvent as by washing, evaporation, or decomposition.

In a preferred embodiment of the invention in which the product comprises the filler particles, the cotton fibers carrying the adhered cellulose ester, and a thermosetting resin of the type of melamine-formaldehyde and phenol-formaldehyde resins, the presently preferred procedure is to first thoroughly wet the filler particles with a solution of the thermosetting resin-forming constituents or with the liquid resin precondensate, in a Hobart mixer, and then slowly add the fibers carrying the cellulose ester or a mixture of such fibers with not more than 50% by weight of other fibers to the wet particles, with mixing. The short fibers tend to curl around the resin-treated filler particles and cling to the surfaces of the particles. The fibers, filler particles and thermosetting resin are uniformly distributed through the resulting mass which is then compacted under heat and pressure to the desired shape.

The mass may be shaped to the desired form in any suitable manner. Thus, the mixture of fibers and filler particles may be introduced into a stationary mold of the desired shape and subjected to heat and pressure in the mold, or it may be continuously forced through a heated extrusion device to produce rods and tubes having any desired cross-section, for example, circular or oval. Under the heat and pressure of the molding conditions, fibers in the mass are bonded together as a result of the adhesiveness of the cellulose ester. The mass obtained by grinding the cotton batting impregnated or saturated with the cellulose ester may comprise loose discrete particles of the ester which may be present in the ground material mixed with the filler particles. Any such discrete fragments of the cellulose ester in the mass molded are activated during the molding step. The activated cellulose ester blinds fibers in the product wherever the ester occurs in it. The products are cooled in or after removal from the mold to deactivate the ester and fix the bonded fibers and filler particles in the bonded relation. Thermosetting resin constituents, if present in the mass molded, are further reacted during the molding step with setting up of the resin which flows to form a film around and between the fibers and filler particles, which film increases the strength of the product. Molded articles comprising the thermosetting resin may be baked at elevated temperatures to fix the resin in the thermoset condition and drive off any water or volatile substances present in the products, the baking being performed at temperatures below the molding temperature.

The present invention may be adapted to the production of compacted fibrous structures comprising particles of filling material and discontinuous fibers of any suitable length. However, in the preferred embodiment the fibers are short, of the order of one-half to one millimeter in length. The cotton batting may be ground (shredded, cut or otherwise broken up) to obtain fibers having a

length in the preferred range and having the cellulose ester adhered to their surfaces as a coating or film, or in the form of discrete particles.

In a preferred embodiment, a reinforcing fabric is associated with the molded fibrous article comprising the discontinuous fibers and filler particles, a fabric, and preferably a woven fabric, comprising a thermoplastic resin or a thermosetting resin in the thermoplastic state being placed over the mass of fibers and filler particles in the mold and bonded to the mass during the molding operation. Fabric woven of nylon yarns may be molded with the mass and bonded to it. The nylon fabric may be coated with a solution of the constituents of a thermosetting resin, or with a partially condensed thermosetting resin, the constituents of the thermosetting resin being reacted while the fabric is in contact with the mass of discontinuous fibers and particulate filler. The fabric need not be woven or otherwise fabricated from yarns of a thermoplastic resin, since fabrics formed from other types of yarns may be coated or impregnated with a thermoplastic resin or with the constituents of the thermosetting resin and molded with the mass of discontinuous fibers and filler particles.

The invention is particularly adapted to the production of various types of abrasive and polishing devices suitable for abrading purposes, including grinding and polishing wheels, abrasive disks, sanding and polishing belts, blocks, pads, and other shapes. Mats or bats comprising the cotton fibers having cellulose acetate adhered to their surfaces, and in which fibers are bonded together, may be cut into squares or sections of any shape to be used in a manner similar to sand-paper or emery cloth, or they may be cut into narrow strips for various purposes. For instance, such mats or bats, or segments thereof, may be glued or otherwise attached to a hand block or the like. Short lengths or pieces of the abrasive mats may be placed in a tumbling barrel with articles which are to be finished, in order to cut down the edges or otherwise polish or finish the exterior of the articles. By incorporating other types of fibers, either potentially adhesive fibers or non-adhesive fibers, or by incorporating both types of fibers with the mass comprising the filler particles and the fibers obtained by grinding or otherwise reducing the cotton batting impregnated with the cellulose ester to a loose fibrous mass, and by controlling the proportion of such fibers present and the extent of activation of the potentially adhesive fibers, the physical properties, such as the softness or hardness of the molded product, can be controlled.

Instead of abrasive particles, particulate filling materials of other kinds may be mixed with the fibers and molded to obtain products having characteristics which adapt them to special uses. For example, molded devices such as washers, caster wheels, wheels for vacuum cleaners, carpet sweepers or the like may be obtained. The use of graphite or similar lubricious types of filler particles results in products which are useful as "oil-less" bearings, washers, packings, etc. For these last-mentioned purposes, the product preferably comprises the thermosetting resin.

The proportion of cotton fibers having the cellulose ester adhered to their surfaces in the product may vary but is usually between 5 and 50% preferably about 25% by weight. The proportion of filler particles may be varied depending upon the type of filler selected and the intended uses of the product, but is usually between 50 and 95% preferably about 65% by weight, when the product consists of the cotton fibers carrying the cellulose ester on their surfaces and the filler. When the product comprises a thermosetting resin, the resin may be present in an amount between 5 and 15% by weight.

By using fibers at least 50% by weight of which are the cellulose ester-treated cotton fibers obtained from the filter media heretofore discarded as a waste product, as the binding fibers in the present products, the invention

provides abrasive and other molded devices which exhibit excellent mechanical and impact strength, at comparatively little expense.

The following examples are given to illustrate specific embodiments of the invention.

#### Example I

A molding mass comprising, on the weight of the mass, 25% of cotton fibers having a length of about one-half millimeter and the surfaces of which carried a film or discrete particles of cellulose acetate (obtained by drying and grinding a cotton batting which had been used to filter a secondary cellulose acetate dope and which was saturated with the dope), 65% of abrasive grit, and 10% of a phenol-formaldehyde resin precondensate was obtained as follows:

The abrasive particles were placed in a Hobart mixer. An aqueous solution of the liquid resin precondensate containing 85% solids was added. After thorough mixing to wet the surfaces of the abrasive particles with the resin, the cotton fibers having cellulose acetate adhered to their surfaces were added slowly and thoroughly mixed with the abrasive. The mass was then placed in the cavity of the female member of a mold provided with a centrally disposed projection and of the type commonly used in molding abrasive wheels. An annular woven nylon fabric was slipped over the central projection of the mold member. The male mold member provided with a centrally disposed hollow projection was placed over the female mold member and pressed upon the nylon fabric and the mixture of fibers and filler particles. Both members of the mold were heated to 350° F. The mass was heated at 350° F. for ten minutes under a pressure approximately 3000 lbs. per sq. in. cooled to deactivate the cellulose ester, and the molded product, a wheel having a diameter of 9" and a central bore having a diameter of  $\frac{3}{4}$ ", was removed. It was placed in a hot air oven and baked at a temperature of 250° F. for four hours to complete the conversion of the phenol-formaldehyde resin to the thermoset, insoluble condition.

#### Example II

A molding mass comprising, on the weight of the mass, 20% of cotton fibers about  $\frac{1}{2}$  mm. long and having cellulose acetate adhering to their surfaces (obtained as in Example I), 5% of fibers of a fiber-forming copolymer of vinyl chloride and vinyl acetate, 65% of abrasive grit, and 10% of a precondensate of a melamine-formaldehyde resin, was obtained as follows:

The abrasive grit was thoroughly mixed with an aqueous solution of the resin precondensate containing 70% solids (available commercially under the trade designation "Resamine 804"), and the cotton fibers and copolymer fibers were added. After thorough mixing, the mass was molded to obtain a wheel which was baked in a hot air oven, all as in Example I.

#### Example III

A molding mass was obtained by mixing 50% by weight of finely powdered pumice with 50% by weight of the cotton fibers obtained by shredding a dried, cellulose acetate-impregnated cotton batting filter, to obtain a loose mass of fibers having a length of about 1 mm. The mass was molded as in Example I to obtain a wheel in which the fibers were bonded together wherever the cellulose acetate occurred in it, and cooled to deactivate the ester and fix the fibers and pumice particles in the wheel.

Since changes may be made in practicing the invention without departing from the spirit and scope thereof, it is to be understood that the foregoing description and examples are illustrative only, and that the invention is not to be limited except as defined by the appended claims.

We claim:

1. A method of making a felt-like, compacted fibrous product which comprises wetting particles of a non-fibrous filler material with a liquid comprising a pre-condensate of a thermosetting resin, associating the wet filler particles with discontinuous cotton fibers having a non-fibrous cellulose organic acid ester adhered to their surfaces, heating the mass of fibers and filler particles to a temperature at which the cellulose ester is rendered adhesive, subjecting the mass to pressure while the ester is in the adhesive condition to obtain a product in which fibers are bonded together by the ester and in which the filler particles are fixed in a condition of substantially uniform distribution by the bonded fibers and by the resin, cooling the product, and heating the product at a temperature below the temperature at which the ester is rendered adhesive to convert the resin to insoluble, thermoset condition.

2. The method of making a felt-like, compacted fibrous product as defined in claim 1 wherein the thermosetting resin is a phenol-formaldehyde resin.

3. The method of making a felt-like, compacted fibrous product as defined in claim 1 wherein the thermosetting resin is a melamine-formaldehyde resin.

4. A felt-like, compacted fibrous abrasive wheel comprising 50% to 95% by weight of abrasive particles,

5% to 50% by weight of discontinuous cotton fibers having a non-fibrous cellulose organic acid ester adhered to their surfaces, and 5% to 15% by weight of a thermosetting resin in the thermoset condition in contact with the abrasive particles, the fibers being bonded together, at least some of the fibers being bonded together by the cellulose ester adhering to their surfaces, and the abrasive particles being fixed in a condition of substantially uniform distribution throughout the wheel by the bonded fibers and by the thermoset resin.

10 5. A felt-like, compacted fibrous abrasive wheel as defined in claim 2 wherein the thermosetting resin is a phenol-formaldehyde resin.

15 6. A felt-like, compacted fibrous abrasive wheel as defined in claim 2 wherein the thermosetting resin is a melamine-formaldehyde resin.

References Cited in the file of this patent

UNITED STATES PATENTS

|           |              |       |               |
|-----------|--------------|-------|---------------|
| 2,398,408 | Buell        | ----- | Apr. 16, 1946 |
| 2,404,207 | Ball         | ----- | July 16, 1946 |
| 2,432,091 | England      | ----- | Dec. 9, 1947  |
| 2,483,406 | Francis      | ----- | Oct. 4, 1949  |
| 2,527,628 | Francis, Jr. | ----- | Oct. 31, 1950 |
| 2,543,101 | Francis      | ----- | Feb. 27, 1951 |